

1

3,846,312  
GREASE THICKENED WITH COATED  
FIBROUS ASBESTOS

Edward A. Cross, Houston, Tex., and Richard L. Frye,  
Baton Rouge, La., assignors to Texaco Inc., New York,  
N.Y.

No Drawing. Continuation-in-part of application Ser. No.  
740,084, June 26, 1968. This application Apr. 30, 1970,  
Ser. No. 33,534

Int. Cl. C10m 5/02, 5/20

U.S. Cl. 252—13

7 Claims

### ABSTRACT OF THE DISCLOSURE

This invention concerns shear stable water-resistant, high dropping point greases having improved E.P. properties comprising a major amount of a lubricating oil thickened with a minor amount of fibrous asbestos coated with at least one polymeric quinoline coating agent.

This invention is a continuation-in-part of Ser. No. 740,084 filed June 26, 1968, now issued as U.S. Pat. 3,520,807.

This invention is related to grease compositions thickened with fibrous inorganic materials coated with hydrophobic materials.

More particularly, this invention concerns lubricating oils thickened to greatest consistency with inorganic fibres coated with at least one polymeric quinoline coating agent.

The use of finely divided fibrous materials such as asbestos or fibrous glass as a filler or thickener in lubricating greases is old in the art. See for example "Manufacture and Application of Lubricating Greases," by C. J. Boner, 1954 edition, pages 757-794, particularly pages 771-773, "Lubricating Greases: Their Manufacture and Use," Klembard, published by Reinhold Publishing Co., pages 725, 756, as well as pages 71, 311, etc. In addition, the subject is also extensively covered in the patent literature, see for example U.S. 3,010,896 (Odell) and U.S. 3,424,678 and U.S. 3,433,743 (Morway et al.). Unfortunately, these greases have been less than satisfactory in one or more respects. For example, the greases alluded to by Boner have poor shear stability and have relatively poor stability in the presence of water. The greases disclosed by Odell comprise water soluble surfactants which must be applied in an aqueous media and require separate and lengthy drying and extraction steps to substantially remove the unwanted water in the system. Further, the resultant greases, while relatively satisfactory, are not superior greases. The two Morway, et al. patents require the use of a particular colloidal size asbestos substrate to be effective.

Recently the applicants have discovered that greases thickened with inorganic fibrous substrates coated with certain polymeric quinoline coating agents overcome the enumerated short-comings of the prior art. For instance, the novel greases have good shear stability and are stable in the presence of water and may be formulated in oils of both natural or synthetic origin. In addition, because of their oil-solubility, the coating agents of this invention can be applied under non-aqueous reaction conditions either *in situ* or preformed and thus obviate tedious and costly dehydration steps in grease manufacture.

In view of the above-recited shortcomings of the prior art, the applicants thickening systems and the greases produced from these systems represent an advance in the art.

It is an object of this invention, among others, to provide novel greases having good shear stability, water resistance and E.P. properties.

2

It is another object of this invention, among others, to provide novel thickening systems applicable to both synthetic and natural oils of lubricating viscosity.

A more specific object of this invention is to provide novel coating agents which can be applied to both colloidal and non-colloidal asbestos substrates in a non-aqueous environment.

Additional objects will suggest themselves to those skilled in the art after reading this disclosure.

10 In practice, a grease is prepared by admixing a major amount of one or more oils of lubricating viscosity and a minor amount of optional adjuvants, with a thickening system comprising

(a) at least one inorganic fibrous material, and  
(b) at least one polymeric quinoline coating agent, under reaction conditions of time and temperature suitable to produce a coating of said polymeric quinoline coating agent upon said inorganic fibrous material until a lubricant of grease-like consistency is obtained. If desired, the grease can be subsequently milled to a harder consistency.

In the favored practice, a grease comprising about 55 to 97 weight percent of a mineral oil of lubricating viscosity and about 45 to 3 weight percent with a thickening system containing inorganic fibrous material and at least one polymeric quinoline is prepared by admixing said grease components at temperatures ranging between about 200° and 450° F. until the desired thickening takes place.

25 30 In the most favored practice, a grease having superior shear stability, water-resistance and extreme pressure properties is prepared by admixing at between about 200° and 450° F. about 65 to 90 weight percent of a mineral oil of the naphthenic or paraffinic type with about 25 to 9 weight percent of fibrous asbestos and about 10 to 1 weight percent of said polymeric quinoline coating agent.

25 35 In the preferred practice, a grease product having superior properties of shear stability, water-resistance and extreme pressure properties is prepared by admixing between about 325° F. and 450° F. the following components:

40 45 about 80 to 90 weight percent of a paraffinic oil having initial viscosities between about 800 SUS to 2000 SUS and about 15 to 9 weight percent of chrysotile asbestos coated with about 5 to 1 weight percent of at least one trimethyldihydroquinoline type polymer having the polymeric unit defined *infra*.

45 50 In order to supplement the subject disclosure of this invention, the following additional disclosure is described more fully below:

55 A. Fibrous Inorganic Materials—The fibrous materials which are suitable as substrates for the novel coating agents of this invention include a wide variety of naturally occurring materials which are found or can be made in the finely divided state and which, under the conditions of formulation, manufacture or application of the grease, are stable to chemical and thermal attack. Most of the materials will range in length from a few millimicrons to tens of thousands of millimicrons, or will range in diameter from fractions of a micron up to about 500 or more microns. More commonly, the lengths will range from about 500 millimicrons to 50,000 millimicrons.

60 65 A useful group of fibrous inorganic materials which are employed as substrates are the siliceous and carbonaceous materials having the requisite stability and size requirements referred to above. These useful favored materials are the various mixtures of alkaline earth metal silicates with other metal and metal oxides, as well as fibrous glass, fibrous carbon and fibrous graphite.

70 75 The favored fibrous materials are the naturally derived silicate mixtures generically referred to as asbestos. They

can be of the long fibered or short fibered type, colloidal or non-colloidal. Asbestos is favored as a class since it is a plentiful, inexpensive material which is relatively stable to chemical and thermal attack which, when coated with the novel coating agents of this invention, are superior thickening agents for converting lubricating oils to greases. The most commonly known types of fibrous asbestos and their theoretical formulae appear below:

Type of Asbestos:

|                     |                                           |
|---------------------|-------------------------------------------|
| Actinolite -----    | $Ca(Mg,Fe)_3(SiO_3)_4 \times H_2O$        |
| Amosite -----       | $(Fe,Mg)SiO_3$ 1-5% $H_2O$                |
| Anthophyllite ----- | $(Mg,Fe)_7Si_8O_{22}(OH)_2$               |
| Chrysotile -----    | $3MgO \cdot 2SiO_2 \cdot 2H_2O$           |
| Crocidolite -----   | $NaFe(SiO_3)_2 \cdot FeSiO_3 \times H_2O$ |
| Tremolite -----     | $Ca_2Mg_5Si_8O_{22}(OH)_2$                |

The information on asbestos presented above, as well as any other data or description relating to asbestos, unless noted otherwise, is taken from the article by M. S. Badollet entitled "Asbestos, A Mineral of Unparalleled Properties," which appeared in *Transactions of the Canadian Institute of Mining and Metallurgy*, Vol. LIV 1951, pages 151-160. As is well documented in the literature, conventional forms of asbestos, particularly asbestos floats, among other forms of asbestos, may be used in greases as long as the particle size falls within the usual size limitations of asbestos fillers. That is, the asbestos may range in length from a few millimicrons to thousands of millimicrons. Similarly, diameters may range from less than a millimicron up to 100 millimicrons or more with a more useful range of diameters being within 10 to 75 millimicrons. While asbestos substrates are favored as a class, as is frequently the case, where the class comprises a large group of entities, some members of the class are more desirable or superior for one reason or another than the rest of the class as a whole, and are therefore preferred. In this instance, the chrysotile form of asbestos is preferred because it is available in an especially high state of purity, substantially free from physical and chemical contaminants, and most important, because when coated with the coating agents of this invention, thicken oils of lubricating viscosity to produce greases having superior properties. Unless otherwise noted, when chrysotile asbestos fibers are referred to in the examples it will fall within the range of properties shown below:

|                           |                                      |
|---------------------------|--------------------------------------|
| Brightness (GE) -----     | 70-80                                |
| Refractive Index -----    | 1.40-1.60                            |
| Dispersion in water ----- | Completely at pH ranges of about 4-6 |
| Surface Area -----        | 14-16 sq. meters/gram                |
| Oil Absorption -----      | 14-16 cc./10 grams of fibers         |
| Water Retention -----     | 20-25 grams per gram of water        |
| Dry Bulk Density Fiber    |                                      |
| Dimensions: -----         | 2-2.5 lbs./cu. ft.                   |
| O.D. -----                | 20-30 millimicrons                   |
| I.D. -----                | 6.0 millimicrons                     |
| Length -----              | 2000-30,000 millimicrons.            |

B. Lubricating Oils—The lubricating oils employed as the base fluid in this invention may be natural (mineral) synthetic or blends of these oils. The mineral oils used are those of the paraffinic, naphthenic, asphaltic or paraffinic-asphaltic type derived from crude oils by refining procedures including distillation, cracking or polymerization. These oils, like their synthetic counterparts, to be described more fully below, will have Saybolt Universal Viscosities in the range from about 75 seconds at 100° F. to about 225 seconds at 210° F.

The synthetic oils will include those of the ester type, the ether type and silicones in the monomeric or polymeric form. The ester type oils are derived from esterifying alcohols, particularly aliphatic alcohols, diols, polyols and the like with organic acids particularly aliphatic mono- and/or dicarboxylic acids. The aliphatic acids ordinarily

contain from 3 to 25 carbon atoms and the alcohol co-reactant ordinarily has from 2 to 20 carbon atoms. Illustrative esters are as follows: diisooctyl azelate, di-2-ethylhexyl sebacate, di-2-ethylhexyl adipate, di-2-ethylhexyl azelate, dilauryl azelate, di-sec-amyl sebacate, di-2-(2-butoxyethoxy) ethyl alkenyl succinate, the di-n-deconate of 1,4-butanediol, the dilaurate of 1,4-hexanediol, the dioctanoate of 1,5-pentanediol, the dilaurate of tetraethylene glycol, the trimethyl propane triheptanoate, the dioctenoate of 1,5-pentanediol and the like.

The lubricating base oils preferred for thickening are mineral oils selected from the group consisting of naphthenic oils having viscosities at 100° F. ranging from about 800 SUS to 2000 SUS and higher. These oils may be derived from blends of oils having lower and higher viscosities. The above oils are preferred as bases for greases, particularly under high pressure conditions because they produce greases particularly resistant to bleeding or separation.

20 C. Optional Adjuvants—The term adjuvant as used throughout this disclosure is used to describe all the materials added to a lubricant to impart or enhance desirable properties or to eliminate or minimize deleterious properties. These materials can be of diverse chemical 25 structure and include oxidation inhibitors, E.P. agents, wear prevention agents, stringiness inhibitors, dropping point improvers and tackiness agents. Illustrative adjuvants are metal oxides, phenyl naphthylamines, mercaptobenzothiazoles, dibenzylsulfides, tricresyl phosphates, chlorinated waxes, fatty soaps, polyalkylene polymers. When adjuvants are employed they seldom total 30 more than 10% by weight of the finished grease and are added at the expense of the lubricating oil component.

D. Polymeric Quinoline Coating Agents—This is the 35 generic term used to describe the oil-soluble or oil-dispersible polymers having recurring units included within the structure:



40 45 wherein  $n$  which represents the average degree of polymerization is from 2 to about 20,  $R$  is selected from the group consisting of hydrogen, alkyl radicals and hydroxylated alkyl radicals, said alkyl radicals preferably containing from 1 to 6 carbon atoms.

50 The above polymers are known materials whose preparation and properties are disclosed in the technical and patent literature. These polymers can be produced among other methods by polymerization monomers obtained from the "quinoline" synthesis which comprises reacting 55 aromatic primary amines such as toluidine or aniline with a carbonyl compound such as acetone or methyl ethyl ketone. For example, the reaction product of aniline and acetone yields 2,2,4-trimethyl-1,2-dihydroquinoline and the reaction of aniline and methyl ethyl ketone produces 60 2-methyl-2,4-diethyl-1,2-dihydroquinoline. Other monomers are 2,2,4,8-tetramethyl-1,2-dihydroquinoline, 2,2,4,7-tetramethyl-1,2-dihydroquinoline, 2,8-dimethyl-2,4-diethyl-1,2-dihydroquinoline, 2,7-dimethyl-2,4-diethyl-1,2-dihydroquinoline and 2,6-dimethyl-2,4-diethyl-1,2-dihydroquinoline among others.

65 The polymerization is carried out by heating monomers of the type described above at moderately elevated temperatures in the presence of a dilute acid. The polymerized materials are also available from a commercial process which comprises heating the monomers between about 110-150° C. in the presence of dilute aqueous hydrochloric acid for at least 16 hours.

70 While generally the above-described class of polymeric materials are suitable coating agents, as is frequently the case in a large group or class, some members of the group

are favored for various reasons to the group or class as a whole. In this instance the favored polymeric coating agents are included within the structure:



wherein  $n$ , which again represents the average degree of polymerization, ranges from about 3 to 6.

The preferred polymeric quinoline coating agents is a commercially available polymer of 2,2,4-trimethyl-1,2-dihydroquinoline obtained from B. F. Goodrich Co. or the Vanderbilt Corporation, consisting chiefly of the trimer, referred to as TMHQ.

E. Processes for Preparing the Inventive Thickening Systems—Two processes are illustrated:

1. *In situ*
2. Preforming

(1) *In situ*—At least two variations are possible in regard to when the coating agent is added. In the first procedure the coating agent is added with the initial charge, while in the second procedure the coating agent is added on the cooling cycle. The following are illustrative of the variations when asbestos, the preferred fibrous substrate is employed.

In the first procedure, the kettle, fitted with heating and agitation means, is charged with lubricating oil, asbestos and the coating agent, and the mixture is vigorously agitated while heating between about 200° to about 400° F. to thoroughly disperse the ingredients. After a heating period of about 30 to 60 minutes the batch is cooled to about 200° to 325° F. by removing the heat source and/or quenching by the addition of lubricating oil. After holding at the reduced temperature for about 30 to 60 minutes, the thickened material is milled through a device such as a colloid mill to the desired consistency.

In the second procedure, the grease kettle is charged with lubricating oil and fibrous substrate and heated between about 200° F. to about 450° F. After heating 30 minutes to 60 minutes, the charge is cooled to between about 200° to 325° F. either by removing the heat source or by quenching the charge with a minor to a major portion of additional lubricating oil. At this time the coating agent is added and the charge is held for about 30 minutes at this temperature and brought to the desired consistency by milling.

(2) Preforming—In this procedure a coated fibrous substrate such as asbestos, previously prepared by either of the two variations described above, is admixed with lubricating oil to be thickened and is heated to about 340° to 405° F. for a period ranging from 5 to 60 minutes. At the end of this time the charge is cooled and brought to the desired consistency.

The *in situ* process for preparing the greases is preferred inasmuch as it requires less handling and shorter process cycles.

F. Preferred Grease Composition—The preferred greases comprise:

- (a) from about 80 to 90 parts by weight of a mineral oil having SUS viscosities at 100° F. ranging from about 800 to 2000 SUS,
- (b) from about 15 to 9 parts of colloidal chrysotile asbestos and
- (c) from about 5 to about 1 parts by weight of at least

one polymeric quinoline coating agent having recurring units included within the structure:



wherein  $n=3$ .

G. Ratio of Thickening System to Grease and Ratio of Fibrous Inorganic Material to Coating Agent Required—The amount of thickening system required is a variable dependent upon a number of factors, primarily the fibrous material and the coating agent employed.

Thickening effects are obtained when the amount of thickening system present comprises from about 1 to 30 parts by weight per 100 parts by weight of final grease product. However, erratic and marginal results are obtained when either of the two extremes of concentration are employed. On the other hand, consistently good results are obtained within a somewhat more restricted range of about 20 to 10 parts by weight of thickening system per hundred parts by weight of grease, and this represents the preferred range. The ratio of fibrous inorganic material to coating agent is a variable dependent upon the fibrous substrate and coating agent employed. Ordinarily the fibrous inorganic material should be present in reasonable excess over the coating agent, that is varying from 1.25:1 to 15:1. When asbestos is the substrate to be coated, favorable results have been obtained when weight ratio of asbestos to the coating material varies between 1.5:1 to 10:1. Inasmuch as the best results have been found in ratios ranging from 2:1 to 7:1, this weight ratio range is preferred.

H. Ratio of Lubricating Oil to Coated Substrate—Generally this ratio is not especially critical. However, favorable results have been obtained when the lubricating oil to coated substrate is between 3:1 to 15:1. When the favored substrate asbestos is used, the preferred weight ratio of lubricant to coated substrate varies from 4:1 to 9:1.

In order to describe the inventive concept in the greatest detail, the following illustrative examples are submitted. Unless otherwise indicated, all parts and percentages are by weight rather than volume.

#### EXAMPLE 1.—MINERAL OIL THICKENED WITH UNCOATED ASBESTOS

An appropriately sized reaction vessel equipped with heating, cooling and stirring means is charged with 13.8 parts by weight of the colloidal chrysotile asbestos described on page 6 and 63.1 parts by weight of mineral oil<sup>1</sup> and heated with stirring to 400° F. The heat is turned off and an additional 20 parts by weight of the mineral oil is added to the stirred reaction vessel to quench-cool to 200° F. At this time the grease is milled to consistency using a colloid mill having a 0.003 inch clearance. As Table I indicates, the resultant grease has unsatisfactory shear stability and water sensitivity properties.

#### EXAMPLE 2.—PREPARATION OF A GREASE THICKENED WITH TMHQ POLYMER

A 96.9 parts by weight portion of the uncoated asbestos thickened grease of Example 1 is charged to a reaction vessel as previously described in the preceding example and heated with stirring at 250° F. Then 3.0 parts by weight of the preferred TMHQ polymer wherein  $n=3$  is added and the mixture is stirred for 30 minutes. As the data in Table I shows, the resultant grease is satisfactory

<sup>1</sup> A refined paraffinic oil having a viscosity of 1600 SUS at 100° F., 117.8 at 210° F. and a flash point of 560° F.

in shear stability and water-resistance showed marked improvement in its performance at high temperature.

**EXAMPLE 3.—PREPARATION OF A LUBRICATING GREASE THICKENED WITH ASBESTOS COATED WITH TMHQ POLYMER**

In this example, the TMHQ coating agent is added during the cooling cycle. The procedure is as follows:

To a reaction vessel equipped as described *supra* is charged 10.8 parts by weight of the mineral oil and 2.25 parts by weight of the asbestos components used in Example 1. The stirred components are heated to 350° F., held there for 30 minutes and quench-cooled by the addition of 1.5 parts by weight of additional mineral oil at 300° F. At this time 0.45 parts by weight of the TMHQ coating agent of Example 2 is added and the batch is held at 300° F. for an additional 30 minutes. Finally an additional 1 part by weight of the mineral oil of Example 1 is added to bring the grease batch to NLGI #1 grade consistency. As can be seen by the data in Table I, results substantially similar to those of Example 2 are obtained.

**EXAMPLE 4.—PREPARATION OF ANOTHER LUBRICATING GREASE THICKENED WITH ASBESTOS COATED WITH TMHQ**

In this example the TMHQ coating agent is added with the original charge. The procedure is as follows. All of the reagents and the apparatus are identical to those described in the previous examples.

A 10.8 parts by weight portion of mineral oil, 2.2 parts by weight of asbestos and 0.45 parts by weight of the TMHQ polymer employed previously, are charged to a reaction vessel and heated with stirring to 350° F. After holding the batch at this temperature for 30 minutes, the batch is quench-cooled to 300° F. by the addition of 1.5 parts by weight of the mineral oil. An additional 4.5 parts by weight of mineral oil is added to the batch to bring it to NLGI #1 grade consistency. An improved yield of grease is obtained, which, as can be seen by the data in Table I, has satisfactory properties.

In all three instances satisfactory greases are produced.

**EXAMPLES 8 AND 9.—GREASES PREPARED USING OTHER INORGANIC FIBROUS SUBSTRATES COATED WITH TMHQ**

Example: Inorganic fibrous materials

8 ---- Fibrous glass described in U.S. Pat. 3,113,105  
9 ---- Non-colloidal chrysotile asbestos described in U.S. Pat. 3,409,499

In both instances satisfactory greases are obtained.

As the specification, including the examples indicate, the novel greases are advantageous in several respects particularly when asbestos is utilized as the fibrous inorganic material to be coated. For example, greases having satisfactory to excellent water-resistance, shear stability and extreme pressure properties are produced when the inventive polymeric coating agents are employed. In addition, the coating agents are relatively inexpensive, commercially available and function at comparatively low concentration levels.

A further advantage of this invention is that numerous changes, modifications and substitutions can be made in the choice of lubricating oils and coating agents without departing from the inventive concept. The metes and bounds of this invention are best gleaned by the claims which follow, read in conjunction with the specification.

We claim:

1. A grease composition having superior shear stability, water-resistance and extreme pressure properties, comprising from about 65 to 90 weight percent of lubricating mineral oil from about 35 to 10 weight percent of a thickening system made up of 25 to 9 weight percent of fibrous asbestos and about 10 to 1 weight percent of polymeric coating agent having recurring units included within the structures:

TABLE I

| Example                                 | 1          | 2     | 3     | 4     |
|-----------------------------------------|------------|-------|-------|-------|
| Composition, percent by wt.:            |            |       |       |       |
| Asbestos                                | 14.3       | 13.8  | 14.1  | 11.5  |
| Mineral oil                             | 85.7       | 83.2  | 83.1  | 86.2  |
| TMHQ                                    | 3.0        | 2.8   | 2.8   | 2.3   |
| Test data:                              |            |       |       |       |
| Penetration:                            |            |       |       |       |
| Unworked                                | 224        | 297   | 206   | 286   |
| Worked 60,000 strokes                   | 355        | 312   | 338   | 333   |
| Worked 100,000 strokes                  | 429        | 310   | 361   | 342   |
| Dropping point, ASTM D-2265-64T, °F.    | 625+       | 625+  | 625+  | 625+  |
| Shell roll, ST-230 points change        | +153       | -34   | -11   | +22   |
| Water absorption, SP-344-60, percent    | 70         | 70    | 70    | 80    |
| Penetration before                      | 278        | 278   | 276   | 265   |
| Penetration emulsion                    | 324        | 291   | 282   | 289   |
| Water washout, 100° F., ASTM D-1264-63% | 1.3        | 3.5   | 5.4   | 6.3   |
| Mean Hertz load                         | 51.6       | 59.3  | ----- | ----- |
| Bomb oxidation, ASTM D-942-50:          |            |       |       |       |
| 100 hrs.                                | 7          | 2     | 5     | 4     |
| 500 hrs.                                | 8          | 7     | 11    | 10    |
| High temp. brg. perf., CRC-L-35-1162:   |            |       |       |       |
| 300° F., hrs.                           | 492; 1,004 | ----- | ----- | ----- |
| 350° F., hrs.                           | 319; 187   | ----- | ----- | ----- |

**EXAMPLES 5 TO 7.—GREASE THICKENED BY ASBESTOS COATED WITH OTHER TMHQ TYPE POLYMERIC QUINOLINES**

Using the procedure, equipment, mineral oil and asbestos described in Example 2, greases are prepared by replacing the 3 parts of the preferred TMHQ polymer with the trimeric quinoline coating agent described below:

Example: Polymeric quinoline coating agent  
5 ---- 2,2,4-triethyl 1,2-dihydroquinoline  
6 ---- 2,4-dimethyl-4-ethyl 1,2-dihydroquinoline  
7 ---- 2,2-di-n-propyl - 4-methyl 1,2-dihydroquinoline



wherein *n* is the average degree of polymerization ranges from 2 to about 20, and *R* is selected from the group consisting of hydrogen, alkyl radicals and hydroxylated alkyl radicals, said alkyl radicals containing from 1 to 6 carbon atoms.

2. The grease composition of Claim 1 wherein the lubricating mineral oil is a paraffinic oil.
3. The grease composition of Claim 1 wherein the lubricating mineral oil is a naphthenic oil.
4. The grease composition of Claim 1 wherein the asbestos is colloidal in size.
5. The grease composition of Claim 1 wherein the asbestos is non-colloidal in size.
6. A grease composition having superior shear stability, water resistance and extreme pressure properties comprising from about 80 to 90 weight percent of mineral oil selected from naphthenic and paraffinic oils having viscosities at 100° F. ranging from 800 SUS to 2000 SUS, from about 15 to 9 weight percent of colloidal size chrysotile asbestos coated with about 5 to 1 weight percent of at least one polymeric quinoline coating agent having recurring units included within the structures:



wherein  $n$  which represents the average degree of polymerization ranges from 3 to 6.

7. The grease composition of Claim 6 wherein the polymeric quinoline coating agent is a trimer.

References Cited

UNITED STATES PATENTS

|           |         |                 |         |
|-----------|---------|-----------------|---------|
| 2,766,205 | 10/1956 | Marshall et al. | 252—50  |
| 2,900,338 | 8/1959  | Postelnek       | 252—50  |
| 3,409,499 | 11/1968 | Dresher et al.  | 252—378 |
| 3,010,896 | 11/1961 | Odell et al.    | 252—20  |
| 3,113,105 | 12/1963 | Slayer et al.   | 252—20  |
| 3,424,678 | 1/1969  | Morway et al.   | 252—20  |
| 3,433,743 | 3/1969  | Morway et al.   | 252—20  |
| 3,520,807 | 7/1970  | Cross et al.    | 252—13  |

DANIEL E. WYMAN, Primary Examiner

I. VAUGHN, Assistant Examiner

U.S. Cl. X.R.

252—28, 50, 51.5 R

UNITED STATES PATENT OFFICE  
CERTIFICATE OF CORRECTION

PATENT NO. : 3,846,312

DATED : November 5, 1974

INVENTOR(S) : Edward A. Cross, Richard L. Frye

It is certified that error appears in the above-identified patent and that said Letters Patent are hereby corrected as shown below:

Column 3, line 51, for "14-16 sq. meters/gram"  
insert -- 45-55 sq. meters/gram --.

Signed and sealed this 20th day of May 1975.

(SEAL)

Attest:

RUTH C. MASON  
Attesting Officer

C. MARSHALL DANN  
Commissioner of Patents  
and Trademarks